

## UNITED STATES PATENT OFFICE

ROBERT SCHLESS, OF EMPORIUM, PENNSYLVANIA, ASSIGNOR TO PENNSYLVANIA POWDER COMPANY, OF EMPORIUM, PENNSYLVANIA, A CORPORATION OF PENNSYLVANIA

## EXPLOSIVE COMPOSITION

No Drawing.

Application filed October 29, 1930. Serial No. 492,092.

This invention relates to explosives, and more particularly to explosive compositions containing high explosives of the nitroglycerin type.

In the low density type of explosives, used to a considerable extent particularly in coal mining and quarrying operations, various types of absorbent carbonaceous materials have been employed. But such explosives have been found as a general rule to be less sensitive to propagation than other types of explosives, especially so upon storage. The reason for this lack of sensitivity appears to reside in the fact that the various carbonaceous materials that have been suggested in the prior art as fillers furnishing the desired bulk, are at the same time very efficient absorbent materials. Their absorptive power far exceeds the capacity necessary to hold in absorption the comparatively low amounts of nitroglycerin contained in the low density types of explosives. As a result of such absorbent properties, the nitroglycerin or other normally liquid high explosive, is held in the cells of the carbonaceous material too tenaciously, and this affects the sensitiveness of the explosives. And this is particularly true on storage of such explosives, since upon storage they become rather difficult to completely detonate, or to propagate the explosion from cartridge to cartridge.

Among the objects of the present invention is the production of explosives, particularly of the high explosive or nitroglycerin type, and within the class of low density explosives, which explosives retain their sensitiveness to a desired degree even upon storage.

Other and further objects and advantages of this invention will appear from the more detailed description set forth below, it being understood however that this more detailed description is given by way of illustration only, and not by way of limitation, since various changes may be made in that more detailed description by those skilled in the art without departing from the scope and spirit of the invention herein described and claimed.

In carrying out the present invention, there is used as the carbonaceous absorbent ingredient, a cereal straw, and particularly a wheat

straw, and especially when in comminuted or in disintegrated condition.

Straw and particularly wheat straw is being utilized today for producing an insulating board product, and in the manufacture of such board material, and particularly after trimming, there remain cuttings or saw dust representing waste material. Such insulating board manufactured from wheat straw is offered in the market under the name of "Inso board", and this particular material is herein-after referred to as "Inso board sawdust". The cereal straw, and particularly wheat straw and also more especially the "Inso board sawdust" have been found to be advantageously useful in explosives as the carbonaceous absorbent materials, since they hold in absorption the required amounts of the liquid explosive ingredients sufficient for practical purposes in explosives of this type, and in addition may serve to supply the combustible material in the process of the extremely rapid combustion called explosion. No separation or exudation of such absorbed liquids occurs even after prolonged storage. And further the comminuted cereal straw acts favorably in retaining to the composition a desired sensitiveness for long periods of time, considerably longer than that possessed by the prior art types of absorbents utilized in this class of explosives. Further, the density of the cereal straw is such that it yeilds explosives of a desirable high cartridge count.

The cereal straw if in satisfactory physical condition requires no particular treatment for employment in the manufacture of explosive compositions. It should, of course, be comminuted, disintegrated, particulated or rasped in order to reduce it to the size of particle desired for this use. In view of the large quantities of "Inso board sawdust" and other material of this character which is readily available on the market, such material comprises a very economical ingredient in the manufacture of explosives. While such cereal straws require no particular further treatment for their use in explosive compositions, they may be given a treatment with various organic or inorganic compounds, such as the compounds employed in explosive com-

positions themselves, for example, sodium nitrate, ammonium nitrate, etc., before being utilized in the preparation of the explosive compositions.

- 5 While nitroglycerin is particularly referred to above in illustrating the types of explosives with which the present invention is concerned, other known substitutes and equivalents of the nitroglycerin may be employed in lieu thereof, or in combination therewith, such as the nitrated sugar-glycerin solutions, nitrated mixtures of glycerin and polymerized glycerin, glycol, and similar compositions.
- 10 In the examples given below illustrating the invention, the substitute or equivalent materials referred to above, or other known substitute or equivalent materials may be used in lieu of those specified in the particular compositions set forth. In addition, in preparing particular types of explosives, some of the stated ingredients may be omitted in accordance with well-recognized practice, or other additional ingredients may be included. These matters are within the skill of those in the art.
- 15 The following examples illustrate compositions embodying the present invention.

|    | I                  | Per cent |
|----|--------------------|----------|
|    | Nitroglycerin      | 15       |
|    | Inso board sawdust | 18       |
|    | Sodium nitrate     | 15       |
| 35 | Ammonium nitrate   | 51       |
|    | Chalk              | 1        |
|    | II                 | Per cent |
|    | Nitroglycerin      | 12       |
| 40 | Inso board sawdust | 11       |
|    | Sodium nitrate     | 10       |
|    | Ammonium nitrate   | 66       |
|    | Chalk              | 1        |
|    | III                | Per cent |
|    | Nitroglycerin      | 10       |
|    | Inso board sawdust | 11       |
|    | Ammonium nitrate   | 76       |
| 50 | Chalk              | 1        |
|    | Salt (common)      | 2        |

The first composition given above yields an explosive having a cartridge count of 195-205, 1 1/4 by 8" cartridges per 50 pounds of explosive, Example II a cartridge count of 180-185, and Example III a cartridge count of about 160.

As illustrated in the examples given above, the proportions of the several ingredients may be varied, and also as noted in the discussions given prior to the examples, some of the ingredients such as the sodium nitrate may be omitted from the composition, or this and other ingredients may be substituted 60 by the recognized equivalents in the art.

Further as noted above, the cereal straw requires no particular treatment prior to its use in the nitroglycerin or other type of explosive compositions. But if desired, the cereal sawdust may be treated with the ammonium nitrate or sodium nitrate for example, which ingredients may be absorbed in the cereal straw prior to the incorporation of the cereal straw in the explosive composition.

Having thus set forth my invention, I 75 claim:

1. A dope for dynamite containing an explosive ingredient and a comminuted cereal straw.
2. A nitroglycerin type explosive containing a comminuted cereal straw as the absorbent.
3. A dope for dynamite containing an explosive ingredient and a comminuted wheat straw.
4. A dope for dynamite containing a comminuted wheat straw as the absorbent.
5. An explosive composition containing a normally liquid explosive, ammonium nitrate and a comminuted cereal straw.
6. An explosive composition containing a normally liquid explosive, ammonium nitrate and comminuted wheat straw.
7. An explosive composition containing nitroglycerin, ammonium nitrate, sodium nitrate, and a comminuted cereal straw.
8. An explosive composition containing nitroglycerin, ammonium nitrate, sodium nitrate, and comminuted wheat straw.
9. A dope for dynamite containing an explosive ingredient and "Inso board" sawdust.
10. A nitroglycerin type explosive containing "Inso board" sawdust.
11. An explosive composition containing nitroglycerin, ammonium nitrate, and "Inso board" sawdust.
12. An explosive composition containing nitroglycerin, ammonium nitrate, sodium nitrate, and "Inso board" sawdust.
13. A composition for use in a dope for dynamite comprising a comminuted cereal straw carrying an absorbed explosives ingredient.
14. A composition for use in a dope for dynamite comprising "Inso board" sawdust carrying an absorbed explosives ingredient.

ROBERT SCHLESS.

120

125

130